

FIP8309

XR 2,395,311

Patented Feb. 27, 1940

2,395,311

## UNITED STATES PATENT OFFICE

2,395,311

## TREATMENT OF WOOD

John C. Woodhouse, Cragmere, and Clarence D. Bell, Wilmington, Del., assignors to E. I. du Pont de Nemours & Company, Wilmington, Del., a corporation of Delaware

No Drawing. Application October 4, 1941.  
Serial No. 413,654

2 Claims. (CL. 117—147)

This invention relates to the treatment of wood and more particularly to color control in chemical seasoning of wood.

In the lumber industry, one of the most serious problems has been that of checking and cracking of wood during its storage and drying after cutting of the timber. This checking and cracking of wood is due, primarily, to the shrinkage resulting from drying of the outer portions of green wood at a more rapid rate than the interior portions. As a consequence of this uneven shrinkage, surface strains and stresses are set up which cause extensive cracking, checking or splitting of the green lumber, being most apparent at the ends and along the surface of the lumber in the central portions of the flat grain cuts.

In the copending application S. N. 353,696, now U. S. Patent 2,302,594, a method is disclosed for overcoming this checking and cracking which comprises, in summary, treating green or unseasoned wood with urea solutions of such concentration, at the particular temperatures employed, that at the wood surfaces the urea solution is completely saturated. In application of the process of Serial No. 353,696, or other methods of applying urea to wood, it has been found that the color change which ordinarily takes place when wood is air-dried or kiln dried is accentuated in some cases, particularly in kiln drying at high temperatures. Some species of wood are much worse in this respect than others and also some species such as oak, when treated with urea and allowed to air season under exposed conditions develop irregular black-brownish areas that penetrate below the normal surfacing depth. These undesired color changes are also found to appear when wood is treated with urea for plasticizing purposes, e. g. when wood is impregnated with urea to an extent such that the wood is thermoplastic.

It is an object of this invention to overcome the drying problems in the lumber industry and to provide a new and improved method for treating or seasoning lumber.

It is a further object of this invention to provide a new and improved method for treating or seasoning lumber with urea without formation of unnatural color in the dried wood.

It is an additional object of the present invention to provide a method for treating wood with urea in such a way that checking and cracking are inhibited and at the same time the wood may be bleached during drying operations.

According to the present invention, wood which is susceptible to cracking and checking during drying or seasoning and which is also susceptible

to darkening and color change upon drying may be inhibited against such checking and cracking, as well as color change, by treatment, prior to drying, with urea and a bleaching agent.

The quantities of urea employed may be varied over a fairly wide range such, for example, as is disclosed in the process described in U. S. Serial No. 353,696, now U. S. Patent 2,302,594, wherein wood is treated with a solution of urea. Although described in detail in the application referred to, this particular urea treatment calls for the use of urea solutions of such concentration that, at the particular temperature employed the urea solution is completely saturated at the wood surface. This invention is not limited to application of urea to wood in the form of solutions, however, for the urea may also be applied to the wood surfaces in crystalline form, as a paste, or the like, the prime requisite being that the urea is applied in the broad range of 5 to 800 pounds per 1000 board feet of wood, preferably from 10 to 200 pounds per 1000 board feet. The quantities of bleaching agent employed may also be varied over a fairly wide range, such as 1% to 20% by weight, based on urea used, 2 to 15% being preferred. Any of the well known bleaching agents may be employed with urea to control the degree of bleaching or color of the final treated wood including peroxides, such as sodium and hydrogen peroxides. Materials which have been found particularly effective, however, according to the present invention, are salts which in solution give ions of bisulfite, hydrosulfite, chlorite, hypochlorite, sulfoxydate, aldehyde sulfoxydate, such, specifically, as sodium and potassium sulfite, sodium and ammonium bisulfite, sodium and potassium hydrosulfite, sodium chlorite, sodium formaldehyde sulfoxydate, zinc formaldehyde sulfoxydate, and the like.

As a further feature of the present invention, we have found that the addition of small quantities of boric acid to the urea-bleaching agent mixture or solution has the effect of increasing the action or wood-lightening effect by the bleaching agent. This effect of boric acid appears to be unique because we have found that wood treated with mixtures of urea bleaching agent and other acids is no lighter in color after seasoning than wood treated with straight urea and bleaching agents. The quantities of boric acid used in any given instance may vary over a fairly wide range such as from 0.25 to 20% by weight based on the urea but we have found that the restricted range of proportions such as 1% to 5% is preferred.

The following examples will illustrate how the

invention may be practiced; parts being given by weight unless otherwise indicated.

#### Example 1

A green  $1\frac{1}{2}'' \times 5\frac{1}{2}'' \times 6''$  Douglas fir sapwood block was surfaced and wet with tap water. A mixture of 100 parts crystal urea and 6 parts sodium bisulfite was applied to the surface of the block at the rate of 42.5 pounds per 1000 board feet. A similar Douglas fir block was placed on top of the urea-sodium bisulfite mixture and the two blocks were stored in a solid pile to permit solution of the urea and sodium bisulfite in the water content of the wood. After two days the blocks were placed in a kiln and dried at  $170^{\circ}\text{F}$ . and 50% relative humidity. Matched untreated blocks and blocks treated only with 40 pounds of urea per 1000 board feet were also kiln dried and surfaced for comparison with the urea-sodium bisulfite treated blocks. The urea treated blocks were brown in appearance, whereas the untreated and urea-sodium bisulfite treated blocks were the natural yellow color of bright Douglas fir sapwood.

#### Example 2

Douglas fir heartwood blocks were treated as in Example 1 except that 2 parts zinc formaldehyde sulfoxylate were used instead of 6 parts sodium bisulfite. The urea-zinc formaldehyde sulfoxylate treated blocks were bleached to a yellow color, whereas the urea treated blocks were slightly darker brown than the untreated Douglas fir heartwood.

#### Example 3

A  $2'' \times 12'' \times 3'$  partially air seasoned white oak board (moisture content about 20%) was cut into one foot lengths. One block was painted with 40% urea solution, one block was painted with 40% urea solution containing 1% sodium bisulfite, and the third block was untreated. The three blocks were then kiln dried at  $140^{\circ}\text{F}$ . and 55% relative humidity. The dried untreated block was normal in color, the urea treated block was dark in color, whereas the urea-sodium bisulfite treated block was brighter in color than the untreated block.

In the above example, the bleaching effect of the bisulfite was confined to the surface. Any desired depth of bleaching and degree of bleaching can be obtained by adjusting the concentration of bleaching agent and the length of time the treated wood is left in solid pile. Increasing the length of time the wood is in solid pile increases the depth of bleaching, and increasing the concentration of bleaching agent increases the degree of bleaching. Great depth and degree of bleaching were obtained in the following test.

#### Example 4

Three separate kiln tests were carried out on random lots of  $2'' \times 6'' \times 6'$  Douglas fir dimension stock containing mixed heartwood and sapwood. Nine pieces were used in each test. The kiln schedule for each test was 24 hours at  $160^{\circ}\text{F}$ . and 80% relative humidity, 22 $\frac{1}{2}$  hours at  $170^{\circ}\text{F}$ . and 60% relative humidity, and 22 $\frac{1}{2}$  hours at  $180^{\circ}\text{F}$ . and 40% relative humidity. Untreated wood was used in the first test. Wood treated with 40 pounds of crystalline urea per 1000 board feet and solid piled 2 $\frac{1}{4}$  days was used in the second test. The wood used in the third test was treated with 36 pounds of crystalline urea and 4 pounds of crystal sodium bisulfite per 1000 board feet and solid piled 5 $\frac{1}{4}$  days. The wood used in the second and third tests was wet with water before applying the crystalline chemicals.

The dried, unsurfaced, urea-sodium bisulfite treated wood was much brighter in appearance than the untreated stock. The bleaching effect extended  $\frac{1}{4}''$  below the surface of the wood, which is greater than the normal depth of surfacing. The urea treated wood was darker in appearance than the untreated.

#### Example 5

Douglas fir heartwood samples  $1\frac{1}{2}'' \times 1\frac{1}{4}'' \times 2''$  were soaked five minutes in an aqueous solution containing by weight 40% urea, 2% sodium bisulfite and 0.5% boric acid. After drying three days in a heated room, the wood was lighter in color than untreated Douglas fir or wood soaked five minutes in a mixture of 40% urea and 2% sodium bisulfite and dried as above.

In the following claims unseasoned wood means wood containing more than about 20% moisture on the basis of the oven dry weight of the wood.

Various changes may be made in the details and preferred embodiments of this invention without departing therefrom or sacrificing the advantages thereof.

We claim:

1. In a process for inhibiting color change of wood during seasoning thereof with urea, the step which comprises contacting the said wood with a composition consisting of 100 parts by weight of urea, 1 to 30 parts of sodium bisulfite and 0.25 to 20 parts of boric acid, the remainder of the composition being water.
2. In a process for inhibiting color change of wood during seasoning thereof with urea, the step which comprises contacting the said wood with a composition consisting of about 40% by weight of urea, about 2% sodium bisulfite, and about 0.5% boric acid, the remainder of the composition being water.

JOHN C. WOODHOUSE  
CLARENCE D. BELL